

## 1

2,919,026

## CONCENTRATION OF POTASH ORES CONTAINING SYLVITE

William Aubrey Smith, Charles W. Abernethy, and Joseph Marshall Downey, Carlsbad, N. Mex., assignors to American Metal Climax, Inc., a corporation of New York

No Drawing. Application August 19, 1955  
Serial No. 529,588

2 Claims. (Cl. 209—167)

This invention relates to the concentration of potash ores containing sylvite and especially to potash ores containing mixtures of oceanic salts and clays and of which sylvite and halite are normal constituents. The invention has for a more particular and representative application the separation and concentration of the sylvite values of sylvinitic ores which in their naturally occurring state contain small but nevertheless objectionable amounts of insoluble clay-like minerals which form slimes that interfere with the concentration of the sylvite content of such ores by flotation and other known concentrating procedures. A typical example of sylvinitic ores of this type is that found in the Carlsbad district of New Mexico.

In concentrating the potash values of such ores by flotation and similar concentrating procedures, it is the general practice to include a preliminary desliming step for removing the objectionable slimes from the ore before it is mixed with the collecting agent that is added to condition the ore for the flotation step. However, it is impractical to effect a complete removal of the slimes by the conventional mechanical methods. Other methods proposed for the preliminary removal of the slimes have so far proven unduly costly in terms of the cost of the reagents, increased investment for additional plant equipment and also increased operating costs.

It has come to be the common practice to effect a preliminary partial removal of the slimes by a mechanical desliming operation and to inhibit the adverse effect of the residual slimes upon the collector by adding an auxiliary reagent in the course of the conditioning of the pulp for the flotation step. Examples of such auxiliary reagents are starch and dextrin, which are most effective when added in a preliminary stage of the conditioning of the ore before the addition of the mineral collector. Other auxiliary agents that have been found to be highly effective for controlling or inhibiting the adverse effect of the clay slimes are the polyglycols and their ethers disclosed in the copending application of William Aubrey Smith, Vernon L. Mattson, Gene Meyer and Robert Baxter, Serial No. 247,384, filed September 19, 1951, now Patent No. 2,724,499.

The present invention is based on our discovery that the use as an auxiliary agent of a member of the herein-after defined group of water soluble acrylonitrile polymers gives surprisingly good results when compared on a quantitative basis with other reagents added for the purpose of inhibiting or controlling the action of the slime on the amine or other conventional cationic collecting agent used in a froth flotation and in generally similar concentration treatments applied to potash ores. The

## 2

polymers that are to be used in practising the present invention are typified by the commercial product sold by Dow Chemical Co. under the trade designation Separan 2610 which is understood to consist essentially of a water soluble acrylonitrile polymer which has undergone partial but incomplete saponification of reactive carboxyl groups. The polymers of this group may be further defined as acrylonitrile polymers in which one or more residual nitrile groups have been modified either by alcoholysis to produce the ester or by alkaline hydrolysis to produce a salt. They are of relatively high molecular weight.

Our investigations also show that when even extremely small additions of the acrylonitrile polymer are made in association with one of the several known auxiliary agents, e.g., one of the polyglycols or their ethers or a polymer consisting principally of mannose units such as guar or a similar mannosgalactan, a distinctly high grade concentrate is produced even when the proportion of the other auxiliary agent is reduced very substantially below the proportion required to be used when such other auxiliary agent is used alone.

The improvement in grade is particularly noticeable when dealing with ore pulps containing considerable proportions of finer particles of sylvite and halite and indicates that the acrylonitrile polymer promotes a greater selectivity of separation of the finer sylvite particles from the finer halite particles so that a smaller proportion of fine halite particles is carried over in the froth collected from the flotation operation. This is a factor of very considerable importance since it furnishes greater assurance that the concentrate will not need to be washed to dissolve out fine halite particles carried over in the froth in order to upgrade the product. When such washing operations have to be applied on occasion in the prior practice in order to upgrade the product there is of necessity a reduction in the recovery of sylvite because finer sylvite particles will be dissolved along with the undesired finer halite particles.

The invention has been found particularly applicable to froth flotation processes but is also applicable to other concentrating operations wherein a selective mineral collector is used.

It is one of the principal objects of the invention to provide an improved method of recovering sylvite from potash ores wherein the usual collector is employed in the flotation step and wherein the acrylonitrile polymer is added as an auxiliary reagent.

It is a further object to provide an improved flotation process employing a mineral collector and an auxiliary reagent wherein a high yield or recovery of the valuable potash constituent is effected with a minimum amount of the auxiliary reagent.

It is a further object to provide an improved flotation process employing a mineral collector and an auxiliary reagent wherein a high yield of the valuable potash constituents in the form of a high grade concentrate is effected.

Other objects and advantages of the present invention will become apparent as the description proceeds.

The results obtained in froth flotation tests conducted on a typical sylvinitic ore from the Carlsbad district are set out in the following tables. In the tests represented

by Table I the ore was crushed and wet ground to minus 8 mesh. It was thereafter screened and washed with a brine saturated with respect to the sylvite and halite constituents until about 50% of the original clay slimes content of the ore was removed. Samples containing approximately 1000 gms. of the thus partially deslimed ore were then conditioned at about 60% solids for one minute with the auxiliary or slime control agents added in the form of aqueous solutions. The amine acetate collector and the frother in the indicated proportions were then added and similarly conditioned for two minutes by thorough mixing with the pulp. The thus conditioned and reagentized pulp samples were then transferred to a Fagergren laboratory flotation machine and diluted to approximately 25% solids. The flotation was then effected at a machine speed of approximately 1000 r.p.m., the froth being removed during an interval of three minutes.

The amine collector used in all of the tests was the commercial product of Armour & Co. sold under the trade designation Armac TD and understood to consist of the water soluble acetate salts of the normal hexadecyl, octadecyl and octadecenyl amines in the approximate proportions of 30, 25 and 45 parts by weight. The frother used was a commercial grade of methyl isobutyl carbitol.

The reagent identified as X-2610 is the commercial product sold by the Dow Chemical Co. under the trade designation Separan 2610 hereinbefore mentioned.

The reagent identified as MPG 750 was the commercial product sold under that designation by Carbide & Carbon Chemicals Co. and is understood to consist of methoxy polyethylene glycol polymerized to a molecular weight of approximately 750.

The reagent identified as "Guar" was the commercial product sold under the trade designation "Guartec" by General Mills Inc. and is understood to consist principally of mannogalactan derived from the endosperm of guar seeds.

The reagent identified as Lytron was the commercial product sold under the trade designation "Lytron 886" by Monsanto Chemical Co. and is understood to be a calcium salt of a carboxyl-containing high molecular weight copolymer of vinyl acetate and maleic anhydride.

Table I

| Test No. | Reagents, Lbs. per Ton Feed |         |               |         | Analysis, Percent K <sub>2</sub> O |      | Percent Recovery of K <sub>2</sub> O equivalent |
|----------|-----------------------------|---------|---------------|---------|------------------------------------|------|-------------------------------------------------|
|          | X2610                       | MPG 750 | Amine Acetate | Frother | Conc.                              | Tail |                                                 |
| 1        | .05                         | 0       | .25           | .04     | 59.8                               | 3.0  | 91.9                                            |
| 2        | .00                         | .25     | .25           | .04     | 59.8                               | 1.20 | 98.7                                            |

In the tests represented by Table II the procedure followed was the same as described for the tests of Table I except that the ore samples used were taken from the flotation feed to an existing full scale plant operation at a point immediately preceding the conditioning stage of the plant operation and after the ore had been subjected to a mechanical desliming treatment that had removed about 50% of the clay slime content of the ore as mined. The solids in this flotation feed were all of a particle size of smaller than 8 mesh and a K<sub>2</sub>O equivalent about the same as the mined ore.

The tests represented by Table II were conducted with the use of Armac TD as the collector and methyl isobutyl carbinol as the frother, with these reagents provided in the same proportions as in Tests Nos. 1 and 2; that is, Armac TD was used in the proportion of 0.25 lb. per ton of feed and methyl isobutyl carbinol was used in the proportion of 0.04 lb. per ton of feed.

| Test No. | Slime Controllant |                  | Analysis, Percent K <sub>2</sub> O |         | Percent Recovery of K <sub>2</sub> O equivalent |
|----------|-------------------|------------------|------------------------------------|---------|-------------------------------------------------|
|          | Identity          | Lb. per Ton Feed | Concen-<br>trate                   | Tailing |                                                 |
| 3        | MPG 750           | 0.10             | 60.17                              | 17.95   | 38.19                                           |
| 4        | X2610             | 0.10             | 56.72                              | 1.56    | 96.44                                           |
| 5        | X2610             | 0.06             | 56.89                              | 3.07    | 92.66                                           |
| 6        | X2610             | 0.028            | 57.88                              | 9.89    | 73.01                                           |
| 7        | Guar              | 0.10             | 58.83                              | 2.45    | 93.96                                           |
| 8        | Guar              | 0.25             | 58.99                              | 3.04    | 92.56                                           |
| 9        | Lytron            | 0.10             | 58.49                              | 16.45   | 45.26                                           |
| 10       | Lytron            | 0.25             | 58.02                              | 2.26    | 94.46                                           |
| 11       | X2610             | 0.014            | 58.28                              | 2.51    | 94.00                                           |
| 12       | X2610             | 0.05             | 57.88                              | 2.69    | 93.57                                           |
| 13       | Guar              | 0.05             | 59.71                              | 9.98    | 72.13                                           |
| 14       | X2610             | 0.014            | 58.65                              | 5.40    | 86.27                                           |
| 15       | MPG 750           | 0.05             | 57.43                              | 2.20    | 94.77                                           |
| 16       | X2610             | 0.20             | 57.70                              | 8.52    | 76.55                                           |
| 17       | X2610             | 0.02             | 58.12                              | 1.38    | 96.92                                           |
| 18       | Guar              | 0.05             | 57.45                              | 1.97    | 95.41                                           |
| 19       | MPG 750           | 0.05             | 57.45                              | 1.97    | 95.41                                           |

Tests Nos. 1-6 show that X2610 is at least several times as effective as MPG 750. When it is borne in mind that MPG 750 is several times as effective as such prior art slime controlants as starch and dextrin it will be understood that the results obtained with the use of X2610 are truly remarkable.

It has also been found, as exemplified by tests Nos. 11-18 inclusive, that the addition of an exceedingly small proportion of X2610 along with one or more of several other auxiliary reagents characterized by their ability to inhibit the adverse effects of the clay slimes brings about a highly successful result even when the proportions of the two or more auxiliary reagents are reduced substantially below those proportions that might be expected to be required if the reagents behaved merely in an additive way. In other words, the association of X2610 with one or more of the other auxiliary reagents seems to produce a synergistic action.

It has been further observed that the use of a partially saponified acrylonitrile polymer of the kind typified by X2610 in association with certain other slime control reagents brings about desirable improvements in the nature of the froth produced in the flotation operation. For example, when the acrylonitrile polymer is associated with a methoxy polyethylene glycol as the auxiliary reagent addition, the froth produced during the flotation operation is less foamy or voluminous than when the methoxy polyethylene glycol is used alone. As a result the flotation action is more selective and there is a lessened tendency for fined particles of the halite to be picked up in the froth and carried over in the concentrate.

It will be understood that in the above tests starvation quantities of the auxiliary reagents were used in many instances for the purpose of emphasizing the contrasts in the action of the auxiliary reagents rather than to produce a commercial result. In other words, the results are not to be understood as representing the maximum recoveries and grades obtainable with the several auxiliary reagents and combinations of such reagents involved.

Although the invention has been described with particular reference to the results obtained when using Separan 2610 as the water soluble partially saponified acrylonitrile polymer, similar results may be obtained with the use of other members of this class.

The beneficial results realized by using various combinations of water soluble partially saponified acrylonitrile polymers of the class defined above with other slime controlants are not confined to the use of the particular additional auxiliary reagents used in the tests herein de-

scribed. Similar results may be obtained by using the defined acrylonitrile polymers in association with other members of the classes represented by MPG 750, Quartec and Lytron 886. For the purpose of this invention the class represented by MPG 750 is to be understood as including the various polyglycols and their ethers having a molecular weight of at least about 300. Likewise in respect of combinations of one of the defined acrylonitrile polymers with members of the class represented by Quartec, it is to be understood that any polymer consisting principally of mannose units may be substituted in place of Quartec; that is, those naturally occurring compounds such as mannogalactan and glucomannan, or any compound in which mannose units are predominant. Similarly in respect of combinations of one of the defined acrylonitrile polymers with members of the class represented by Lytron 886, it is to be understood that any relatively high molecular weight vinyl acetate-maleic anhydride co-polymer may be used in the combinations. These co-polymers are available in their purely organic form and also as their alkali metal and alkaline earth metal salts.

The invention may be practiced with similar advantage when using any of the various cationic collectors known to be effective in floating sylvite and similar potash values from potash ores and is not limited in its application to the use of an amine collector. It is also to be understood that other frothers than methyl isobutyl carbinol may be used in the process. Other representative examples are methyl amyl alcohol and pine oil.

The invention has been found particularly applicable to froth flotation processes, but is adaptable to other wet

stratifying processes such as skin flotation and agglomeration tabling.

We claim:

5 1. The improvement in the separation of sylvite from potash ores containing sylvite in association with minor but objectionable amounts of clay slime-forming constituents by a concentrating process employing a cationic mineral collector which comprises forming a pulp of said ore by suspending the ore in a saturated aqueous solution of the soluble ore constituents, distributing in said ore in advance of the addition thereto of the cationic mineral collector a plurality of auxiliary agents, one of which consists essentially of about 0.02 lb. per ton of said ore of a water soluble acrylonitrile polymer in which at least one nitrile group has been modified by a process selected from the group consisting of alcoholysis to produce an ester and alkaline hydrolysis to produce a salt, and another of which consists of about 0.10 lb. per ton of said ore of a member having a molecular weight of at least about 300 selected from the group consisting of polyglycols and their ethers.

10 2. The improvement in the separation of sylvite from potash ores according to claim 1 wherein said member is methoxy polyethylene glycol of a molecular weight of approximately 750.

References Cited in the file of this patent

UNITED STATES PATENTS

|    |           |                     |               |
|----|-----------|---------------------|---------------|
| 30 | 2,696,912 | Atwood et al. ----- | Dec. 14, 1954 |
|    | 2,724,489 | Smith et al. -----  | Nov. 22, 1955 |
|    | 2,740,522 | Aimone et al. ----- | Apr. 3, 1956  |